

1,235,598.

A. RAMÉN.  
METHOD FOR TREATING ROASTED ORES WITH LIQUIDS.  
APPLICATION FILED MAR. 4, 1915.

Patented Aug. 7, 1917.

FIG: 1.



FIG: 2.



WITNESSES:

John C. Sanders  
Bradley S. Howard

INVENTOR:

Arthur Ramen  
By  
John Muller Milt

# UNITED STATES PATENT OFFICE.

ARTHUR RAMÉN, OF OLYMPIA, HÄLSINGBORG, SWEDEN.

## METHOD FOR TREATING ROASTED ORES WITH LIQUIDS.

1,235,598.

Specification of Letters Patent.

Patented Aug. 7, 1917.

Application filed March 4, 1915. Serial No. 12,010.

To all whom it may concern:

Be it known that I, ARTHUR RAMÉN, a subject of the King of Sweden, residing at Villa Skansen, Olympia, Helsingborg, Sweden, have invented new and useful Improvements in Methods for Treating Roasted Ores with Liquids, of which the following is a specification.

The present invention relates to a method 10 of treating roasted ores for the purpose of facilitating their subsequent lixiviation.

If for instance a chloridizing roasted ore is lixiviated in the hitherto used manner in vats or basins, it will harden or form 15 larger or smaller agglomerates or lumps, whereby the lixiviation is highly retarded and large quantities of lixiviating liquid are needed. The formation of such lumps or agglomerates is due to the fact, that all the 20 particles of the ore have not been treated with equal quantities of liquid, some particles absorbing the liquid more rapidly than the other ones. These particles also 25 become lixiviated easier than the other ones at a subsequent lixiviation, because the liquid can pass better through them than through the other ones, so that it will be formed in the whole bulk of the ore channels or passages, through which the lixiviating 30 liquid preferably passes, while other portions of the ore become acted upon by the said liquid in a relatively little degree. For that reason the lixiviating liquid must be used in a very great excess, and the time 35 of lixiviation must be very long if a complete lixiviation of the roasted ore shall take place.

If ores, having been subjected to a chloridizing roasting, are treated in the manner 40 hereinafter described and forming the object of the invention, with a suitable quantity of liquid (which quantity shall only be such that the ore becomes intimately mixed therewith without any great excess of the 45 liquid in the mixture) and if the said treatment is carried out before the ore is brought to the vats or basins, in which the usual lixiviation takes place, the advantage is gained, that the ore during this lixiviation 50 does not form agglomerates or lumps, (counteracting a complete and rapid lixiviation), because all the particles of ore already from the beginning of the treatment 55 are treated with even that quantity of liquid, which they are able to absorb, whereby the said particles have changed their

physical qualities and lost their disposition of absorbing different quantities of liquid and of forming hard lumps or agglomerates. For this reason, any formation of lumps 60 and agglomerates is avoided, and the whole mass will be completely porous and penetrable for liquid which is not otherwise the case. At a following lixiviation in vats or basins of ore thus treated the process can 65 be effected in a fraction of the time which is otherwise necessary, because no hard agglomerates have been formed which require longer time for lixiviation; the solutions obtained also will be concentrated. 70

The liquid used for treating the ore cools it, if the ore is hot, for which reason the ore at the lixiviation in the vats or basins is cool and cannot cause any formation of dust and steam, which formation now takes 75 place at the treatment with the liquid now mentioned, whereby the collection of dust, gas and steam in any suitable manner becomes possible without difficulty.

The method consists in that the roasted 80 ore, spread in a thin layer on a movable bed not permeable to liquid, is sprinkled or sprayed as it is fed forward, by a quantity of liquid distributed over the width thereof, while at the same time the dust and vapors 85 which may be formed when the hot ore is sprinkled with the liquid can be carried away by suction to a condenser in which the gases are condensed by means of liquid while the ore particles are suspended in the 90 condensed product from which they are afterward filtered off.

In the accompanying drawing, a device suitable for carrying out this method is shown in a side view in Figure 1 and in a 95 plan view in Fig. 2.

The apparatus illustrated in Figs. 1 and 2 consists of a feeding hopper *a* for the roasted material, the lower mouth of said hopper situated at a short distance above a rotating bed, formed as a plate or table *b*. The hopper should be adjustable vertically so as to control the thickness of the ore layer fed down upon the table. In front of the hopper, as regards the direction of rotation of the table, is a pipe *c* with several small openings, through which water or other liquid may be sprinkled over the hot material, fed forward in an even layer over the table, said material being then evenly treated with the liquid so as to be cooled and transformed in a more easily extractable 110

state. *d* is a hood or casing suitably arranged around the apparatus (shown in dash and dotted lines) and serving to prevent the formed vapors and dust from spreading; said casing should be provided with a pipe *e* leading to a condenser *f* on the bottom of which the ore particles are collected. The hot water (or liquid) obtained by condensation of liquid in the condenser is conducted off alone at *g* and used for instance for lixiviating ore in extracting whereby the heat taken from the ore is utilized. The non-condensed gases are conducted off at *h*. The ore on the table is carried, during the rotation of said table, toward a scraper *i* which removes it from the table through an opening in the casing.

If the ore is not subjected to the liquid in a hot condition no vapors are formed and the casing can be omitted.

The sprinkling with liquids of substances placed upon a movable filter bed for lixiviation, extraction or washing of them is known. According to the present invention 25 a movable bed is used not for lixiviation, but for the mixing of the roasted ore with a liquid, so that all the particles of the ore become uniformly treated and are uniformly altered as to their physical or chemical qualities, whereby better results are obtained at the subsequent lixiviation.

By exactly suiting the quantity or the nature of the liquid used in such treatment of roasted ore some of the salts present in the 35 roasted ore can be transformed into a more readily soluble state than other ones. By successive lixiviation of the ore thus treated there may thus first be obtained a solution which chiefly contains the more soluble salts 40 and then a solution containing the less soluble ones.

It is possible in the manner now described to treat efficiently ores containing substances which have been transformed, by chloridizing 45 or other roasting, into a form soluble in certain solvents or originally are present in the ore in this form. Thus for instance ore containing silver which has been transformed into silver chlorid by chloridizing 50 roasting can be treated with a solution of common salt or hyposulphite, or, if containing gold, with chlorinous water, it being then possible to treat all the particles with equal 55 quantities of solvent which thus need not be added in excess. In a similar way other solvents may be employed or such liquids which are obtained at the extraction of ores treated according to the present method.

In the manner now described it is easier 60 than before to utilize for instance zinc from the solutions or lyes obtained in extracting roasted copper ore containing zinc. As the copper, for economical reasons, is generally precipitated from the lyes by means of iron 65 which then is partially dissolved, the final

lye will contain the zinc mixed with iron which must be removed for making the zinc capable of being used. By treating copper ore which has been subjected to chloridizing roasting in the above described manner, the zinc during the following complete lixiviation of the ore may first be extracted in one lye and the copper in a following one. In the first lye then a quantity of copper will be present, but so small that only a very small 75 quantity of iron will be required for precipitating it. For this reason, very small quantities of iron are dissolved in the zinc solution compared with the quantities obtained in the usual processes, and these 80 quantities therefore can easily be removed, compared with the large quantities of iron present in the solutions after precipitating the copper by iron from solutions containing zinc according to the usual process.

It is obvious that similar advantages are obtained in utilizing zinc solutions even if another precipitating agent for copper than iron is used.

For controlling the quantities of liquid 90 and ore the speed of the carrier may be made adjustable.

Having now particularly described the nature of my invention and the manner of its operation, what I claim is:

1. The method of treating roasted ores which consists in continuously feeding the ore in a thin layer upon a movable impermeable bed, sprinkling the layer uniformly with a quantity of liquid, removing the ore and absorbed liquid from the bed, and lixiviating the same.

2. The method of treating roasted ores which consists in continuously feeding the ore in a thin layer upon a movable impermeable bed, sprinkling the layer uniformly with a quantity of liquid, removing by suction the gases, vapors and dust formed during the sprinkling, removing the ore and absorbed liquid from the bed, and lixiviating the same.

3. The method of treating roasted ores which consists in continuously feeding the ore in a thin layer upon a movable impermeable bed, sprinkling the ore uniformly 115 with a quantity of a liquid adapted to render some constituents of the ore more soluble than others, removing the ore and absorbed liquid from the bed, and lixiviating the same.

4. The method of treating roasted ores which consists in continuously feeding the ore in a thin layer upon a movable impermeable bed, sprinkling the ore uniformly with a quantity of a liquid adapted to render 125 some constituents of the ore more soluble than others, removing by suction the gases, vapors and dust formed during the sprinkling, removing the ore and absorbed liquid from the bed, and lixiviating the same.

5. The method of treating roasted ores which consists in feeding the ore in a thin layer upon a movable impermeable bed, sprinkling the ore uniformly with a quantity of liquid, removing by suction the gases, vapors and dust formed during the sprinkling, removing the ore and absorbed liquid from the bed, and subjecting it to repeated lixiviations for obtaining different lyes.
- 10 6. The method of treating roasted ores which consists in feeding the ore in a thin layer upon a movable impermeable bed, sprinkling it uniformly with a quantity of a liquid adapted to render some constituents

of the ore more soluble than others, removing by suction the gases, vapors and dust formed during the sprinkling, removing the ore and absorbed liquid from the bed, and subjecting it to repeated lixiviations for obtaining different lyes.

15 In testimony whereof I have signed my name to this specification in the presence of two subscribing witnesses.

ARTHUR RAMÉN.

Witnesses:

ADA SIMON,  
H. HAMMAL.